



# United States Patent Office.

WILLIAM W. HARDING, OF PHILADELPHIA, PENNSYLVANIA.

*Letters Patent No. 86,012, dated January 19, 1869.*

## IMPROVEMENT IN THE MANUFACTURE OF PRINTING AND WRITING-PAPER.

The Schedule referred to in these Letters Patent and making part of the same.

*To all whom it may concern:*

Be it known that I, WILLIAM W. HARDING, of the city of Philadelphia, and State of Pennsylvania, have invented a new and useful Improvement in the Manufacture of Printing and Writing-Papers; and I do hereby declare the following to be a full and exact description of the same.

The nature of my invention consists in coating both sides of a sheet of paper with an opaque sizing, and then calendering it on both sides.

I take a continuous sheet of ordinary paper, and then apply, by means of a revolving brush, or revolving felt roller, an opaque liquid sizing, to each side of the sheet of paper. This sizing is then dried thereon, by passing the sheet through a heated chamber, or by passing it over a heated cylinder covered with cloth or felt. The sheet is then passed between a double set of heated or cold calender-rollers, and each side will be calendered.

I make a good opaque size of one pound of glue, or gelatine, and ten pounds of china-clay, five pounds of blank fix, (sulphate of baryta,) one pound of linseed-oil, or other similar oil, and about fifty pounds of water. Instead of oil, wax or stearine may be used in the same proportion. Any tinting-material may be added, if desired.

The advantage of this invention is that low-priced paper, with an inferior or discolored surface, can be

converted into writing or printing-paper, having a fine finished white or tinted surface on both sides.

Instead of the opaque size above mentioned, other opaque size compound, of glue, clay, or other well-known ingredients for making liquid enamel, might be substituted.

Having thus described by improvement,

What I claim, is—

1. The process of treating papers by applying opaque size to both sides, to give a surface-color to both sides, independent of the body of the paper.

2. The process of making writing or printing-paper by applying opaque size to both sides, and then drying and calendering it on both sides, so as to impart to inferior paper a surface having a fine finish and surface-color on both sides, independent of the color and finish of the body of the paper so treated.

3. As a new article of manufacture, writing or printing-paper, made in a single sheet, and then coated on both sides with opaque white or tinted size, for imparting color and finish to the two surfaces of the sheet, independent of the color or surfaces of the original sheet.

WM. W. HARDING.

Witnesses:

WM. H. SOLEY,  
GEO. E. BUCKLEY.